

## UNITED STATES PATENT OFFICE

2,015,424

PROCESS FOR SURFACING ELECTRODES  
FOR ELECTRICAL-DISCHARGE TUBES

Albert C. Forst, Alameda, Calif.

No Drawing. Application July 26, 1932,  
Serial No. 624,909

2 Claims. (Cl. 176—126)

The invention relates to processes employed in cleansing and coating the metal surfaces of electrodes, such as employed in electrical-discharge tubes, for the purpose of rendering these surfaces more efficient in their operation on the electrode.

The essential purpose of treating and coating electrode surfaces by processes of the class here disclosed is to render these surfaces of such a nature that they may cooperate most effectively with the shape of the electrode to support about the latter an electrostatic field that will cause a confinement of the electrical discharge to a relatively small portion of the surface and at the same time prevent corona and other undesirable discharge from occurring over the remainder of the surface. Such a surface treatment usually comprises covering the entire electrode, other than a relatively small portion, with an insulation coating and rendering the uncoated portion of a nature to withstand sustained electronic bombardment without materially affecting its conductivity. Processes for carrying out such a surface treatment have been used on electrodes of certain metals, especially copper and iron, but to my knowledge none of these processes has been successful when applied to a metal such as aluminum. This latter metal has many inherent qualities of advantage over both copper and iron, particularly in its availability in a substantially pure form that is remarkably free from impurities and excessive quantities of entrapped surface gases which when released in a gaseous electrical discharge tube harmfully disturb the character of the light emitted. It therefore forms one of the principal objects of my invention to provide a process of the character aforesaid which may be especially and efficaciously applied to electrodes of aluminum.

Another object of the invention is to provide a process of the character described which will substantially completely liberate gases entrapped in the surfaces of the electrode and thereafter seal the surfaces against reabsorption of such gases.

A further object of the invention is to provide a process for treating and coating the surfaces of electrodes which will materially increase the ability of such surfaces to withstand intense heat as well as heavy electronic bombardment over long periods of use.

The invention possesses other objects and features of advantage, some of which, with the foregoing, will be set forth in the following descrip-

tion of the preferred form of the invention. It is to be understood, however, that variations in the showing made by the said description may be adopted within the scope of the invention as set forth in the claims.

In accordance with the process of my invention, it is desirable to first effect a thorough cleaning of the electrode surfaces to be coated, and for this purpose the electrode is boiled in water from ten to thirty minutes to remove the soluble surface impurities and to cause any oil or grease present on the electrode to be dislodged and separated therefrom, the free oil and grease naturally rising to the surface of the water from where it may be removed. After being initially cleaned in this manner, the electrode is removed from the water without contact with the oil or grease and placed in a bath of oxalic acid, diluted with about four parts water, and left in the acid from four to twelve hours.

The action of the acid on the aluminum is to form a film of aluminum oxide over the surface of the electrode, and such action is allowed to continue until the surface of the electrode loses its gloss and becomes definitely dull in appearance, thereby signifying a sufficient accumulation of the oxide. The electrode on being taken from the acid bath is rinsed in cold water, dried and then heat treated to cause a fusion of the oxide on the surface of the metal. The heat treatment may be effected either by contacting the electrode directly with a clean flame or placing the same in a suitable oven and gradually raising the temperature of the electrode to a dull red heat, after which the electrode is removed from the presence of the heat and allowed to cool.

The fused oxide surface serves a dual purpose for it not only forms an excellent conducting surface for the discharge emitting portion of the electrode, but also provides a secure base upon which an insulating covering may be mounted. The incorporation of such a covering on aluminum has in the past been one of the major problems in the use of electrodes of this metal. In accordance with my process, however, having provided a fused oxide base upon which to build, I proceed by coating this base, with the exception of the area providing the discharge portion of the electrode, with a vitreous enamel and again subject the electrode to a relatively high heat in order to fuse the enamel into a glaze thereby forming an insulation covering over the surface of the electrode. Any suitable low fusing vitreous glaze using finely ground glass, porcelain or lava

as a base may be used. The heat treatment of the surface for fusing the glaze may in the first instance be carried out either over a flame or in an oven, and the temperature of the surface is preferably raised to a dull red heat and thereafter allowed to cool. The final heat treatment in addition to fusing the enamel serves to liberate surface gases on the electrode and fuse the enamel into surface sealing relation which checks reabsorption of the gases upon cooling of the surface.

With the surfaces of the electrode thus freed from and sealed against absorption of surface gases and impurities, the probable quantity of inert gases and foreign material other than the rarified gas in an electrical discharge tube may be accurately determined and depended upon to remain constant over long periods of use. Formerly it was necessary during the filling of the tube with the rarified gas to not only include sufficient of the latter to subdue the effects of the foreign gases and impurities present at the outset, but in addition supply an over-abundance of such rarified gas to overcome the effects of foreign gases and other impurities which are subsequently liberated by the electrodes after the tube has been in operation for some time. This

latter quantity of gas which is added with the expectancy of satisfying subsequent gaseous conditions in the tube has in the past been a source of much waste and uncertainty. In accordance with the process of my invention, however, it will be apparent that the electrodes are so surfaced and treated as to substantially entirely prevent the subsequent liberation of foreign gases or impurities, and therefore enable the use of a minimum and absolutely consistent quantity of rarified gas, thereby effectively serving to eliminate the aforesaid waste and uncertainty.

It will now be clear that the process of my invention is well adapted to the accomplishment of the objects hereinbefore referred to.

I claim:

1. A process for surfacing aluminum electrodes for gaseous electrical discharge tubes which comprises treating said electrode with oxalic acid, thereafter heating said electrode to dull red heat and cooling, and thereafter fusing onto said electrode a vitreous coating.

2. An electrode for gaseous electrical discharge tubes of neon and the like comprising, an aluminum member having a base surface coating of a fused layer of aluminum oxide, and an outer layer of a fused vitreous substance.

ALBERT C. FORST.